# EUROPEAN PATENT APPLICATION

(11) **EP 0 738 799 A2**
(43) Date of publication of application: **23.10.1996**
(21) Application number: 96500004.5
(22) Date of filing: 10.01.1996
(51) Int. Cl.: D06M 13/127, D06P 1/651, D06P 3/79

(54) **Method for dyeing and finishing of garments made of polypropylene**

(30) Priority: 12.01.1995 ES 9500047
(71) Applicant: Falguera Xifra, José, 17800 Olot (ES); Sacrest Villegas, Ramon, 17800 Olot (ES); Tomas Riba, Josep, 17800 Olot (ES)
(72) Inventor: Tomas Riba, Josep, E-17800 Olot (ES)
(74) Representative: Marques Alos, Fernando

(57) **Abstract**

PROCEDURE FOR DYEING AND FINISHING OF GARMENTS MADE OF POLYPROPYLENE, characterized by the fact that it comprises four phases, the first being preparation of the garments 1, in which they are dipped in formaldehyde 2 dissolved in water; the second phase consisting of dyeing 5, where the garments are immersed in water 6 with a dissolved Cryogen or sulphurus type colouring agent 7, immediately adding a reducing agent 8, such as sodium hydrosulphite, after which an electrolyte 9 is added, consisting of Sodium Chloride; the third phase consisting of oxidation 11, during which the garments are dipped in a solution of water 18 with a dissolved acid and oxidant agent 12; the final phase is the finishing 15, when the garments are immersed in a water bath 16, in which a softening agent 17 has been dissolved, consisting of a liquid polyamide of animal origin.

## Description

### DESCRIPTION OF THE INVENTION

The object of this invention, as it is expressed in the statement of the following descriptive report, consists of a PROCEDURE FOR DYEING AND FINISHING OF GARMENTS MADE IN POLYPROPYLENE.

Garments made with polypropylene fibres offer a series of benefits, such as the lack of abrasive properties, they cannot become misshapen, they shrug off water and odours, and they are recyclable.

However, production of garments in polypropylene is limited to a small range of colours in which the manufacturers of polypropylene fibres supply their product.

In order to expand the range of colours with which fashion designers work, the fibres or the ready-made garments need to be dyed.

Conventionally, dyeing a fibre is effected by dipping the garments in a solution containing colourant molecules and appropriate reagents, as a result of which these molecules penetrate the fabric and are fixed to it. New pigments are thereby incorporated into the fibres, giving them a colour other than the original.

However, polypropylene, being a non-hydrophilic fibre, shrugs off any kind of molecule and therefore does not allow the pigments to penetrate inside by the conventional dyeing process, which is based precisely on the hydrophilic nature of the fibres.

Polypropylene can only be coloured during manufacture in its mass form, before being converted into fibre, and, once its bonds are established, it can no longer be modified in the same way as other fibres.

The new process for which a patent is sought, manages to retain the molecules of colourant inside the polypropylene fibres, and in this way the colour of the garments can be altered, thereby providing a spectacular increase in the range of colours with which designers and manufacturers can produce their creations in this material.

Essentially, the process begins with preparation of the garments, which are dipped in formaldehyde dissolved in water, for a period of time which, depending on the colour to be used, varies between 10 and 20 minutes, at a temperature of between 40ºC and 80ºC. The formaldehyde is in a proportion in weight in relation to the polypropylene fibre of between 1 and 5%, depending on the colour, and the water, in a proportion of 10 litres per garment.

This dip provides a film of formaldehyde which covers the surface of the polypropylene fibres.

Next, the garments are washed, in order to remove any excess formaldehyde, as formaldehydes have an unpleasant odour and any excess would cause problems in the evenness of the garment.

Next, the colourant is applied.

This colourant must be Cryogen or Sulphurous, and its application is effected in a water bath of 10 litres of water per garment, in which, subsequent to application of the colourant, a reducing agent, such as sodium sulphydrate or sodium hydrosulphite, is added, in a proportion of 1 to 3% in relation to the weight of the polypropylene fibre.

This reducing agent causes the molecules of colourant to subdivide, producing thousands of molecules which are very much smaller, which can penetrate the polypropylene fibres and displace themselves inside these.

This bath is left for between 10 and 30 minutes at room temperature and, after this time, the bath temperature is raised to end at between 50ºC and 70ºC, at which point common salt is added to the solution.

In view of the fact that polypropylene fibre does not absorb much, the common salt buffers the solution, preventing the split molecules of colourant which have not penetrated into the fibre and which are, therefore, excess, from becoming deposited on the surface of the garment, as they are destroyed by the saturation of the water with salt, thereby leaving the garments clean.

At this point, the garments and, consequently, the fibres of which they are made are now dyed and displaying their new colour; they are now again washed with water in the same proportion of 10 litres per garment.

Next, the garments are poured into a solution of hydrogen peroxide diluted to 200 volume and an acid such as acetic acid, which acts as a catalyst so that the oxygen in the hydrogen peroxide is given off and oxidizes all the molecules of colourant which were in a reduced state inside the polypropylene fibre, increasing the size of these molecules and completing the bonds between the polypropylene fibres and the colourant, which is thereby finally fixed to the fibre.

This phase is carried out at a temperature of between 40ºC and 60ºC, for 15 to 30 minutes.

Next, the garments are subject to two consecutive washes with non-ionic detergents, at a temperature of 40ºC for 15 to 20 minutes each, whereby the molecules of colourant which have not been able to be fixed to the fibre are eliminated.

Finally, the garments are softened using an animal substance, preferably fatty acid or any amphoteric substance, and denatured alcohol, for 10 to 20 minutes at a temperature of 60ºC to 80ºC, whereby the new process for dyeing polypropylene fibres and garments is concluded.

### DESCRIPTION OF THE SKETCHES

In order to illustrate the foregoing, a sheet of sketches representing a diagram in blocks, corresponding to the dyeing process as per the claim, is attached to this descriptive report, forming an inseparable part of same.

### DESCRIPTION OF A PRACTICAL CASE

This practical case is concerned with dyeing 100 polypropylene garments, with an overall weight of 70 kg.

As per the invention, the dyeing process is begun with the preparation or mordant of the garments 1.

The garments are put into a washing machine type, exhaustion, garment-dyeing machine, together with 5% formaldehyde (applied in gr/l) 2, dissolved in 700 l. of water 3. This phase is effected at a temperature of 40ºC and lasts 15 minutes.

After this phase, the garments are washed with water 4 to eliminate the excess formaldehyde.

The second phase is for dyeing 5, for which the garments are immersed in 700 l. of water 6, in which a Cryogen type colourant 7 has been dissolved, in a ratio of 15% to 30% of the weight of the matter to be dyed, and next a reducing agent 8 is added, consisting of sodium hydrosulphite in a ratio of 2% of the weight of the matter. This bath is left for 30 minutes at room temperature, after which an electrolyte 9 is added to the solution, consisting of Sodium Chloride, in a ratio of 20 gr/l, and the temperature is raised to 65ºC and kept like this for a further 45 minutes. After this time, the garment are washed again with water 10.

At this point, a third, oxidation phase 11 is begun, where the garments are dipped in 700 l. of water 18, in which an oxidant agent 12 has been dissolved, consisting of 200V hydrogen peroxide in a proportion of 3% gr/l. This operation is carried out at 50ºC and is left for 20 minutes, after which the garments are washed again, twice in a row, 13 and 14.

After these two consecutive washes, the finishing phase 15 is begun, where the garments are immersed in 700 l. of water 16, in which a fatty acid derivative, anionic type, softening agent 17 has been dissolved, in a proportion of 2% of the weight of the matter, and this last dip is effected at a temperature of 80ºC and lasts 20 minutes, after which the 100 garments will be completely finished.

Having provided the description to which the foregoing report refers, it is necessary to stress that the details of execution of the idea set out may undergo minor alterations, although always based on the fundamental principles of the idea, which are essentially those set out in the paragraphs of the description provided.

Having established the aforesaid concept, there follows the text of the claims note, thereby synthesizing the new processes to be claimed:

### NOTE

In sum, the privilege of exclusive exploitation which is applied for will be based on the following claims:

## Claims

1. **"PROCEDURE FOR DYEING AND FINISHING OF GARMENTS MADE IN POLYPROPYLENE**", characterized essentially by the fact that it consists of four phases; the first being the preparation or mordant of the garments 1, where the garments are dipped in formaldehyde dissolved in water, in a proportion of approximately 10 litres of water per garment 3 and 1% to 5% of formaldehyde applied in gr/l. 2, and this dip is effected at a temperature of between 40ºC and 80ºC for a period of between 10 and 20 minutes, after which the garments are washed with water 4 to eliminate the excess formaldehyde, and the second phase begins, consisting of the dyeing 5, where the garments are immersed in water 6, in which a Cryogen or sulphurous colourant 7 has been dissolved in a ratio of 15% to 30% of the weight of the matter to be dyed and next, a reducing agent 8 is added, consisting of sodium hydrosulphite or sodium sulphydrate, in a ratio of 1% to 3% of the weight of the matter, and this dip is left for 10 to 30 minutes at room temperature, after which an electrolyte 9 is added to the solution, consisting of Sodium Chloride, in a ratio of approximately 20 gr/l., and the temperature is raised to between 50ºC and 70ºC and left in these conditions for approximately 45 minutes, after which the garments are washed again with water 10, at which point the third phase begins, consisting of oxidation 11, where the garments are dipped in a solution of water 18, in which an acid has been dissolved, such as acetic acid, and an oxidant agent 12, consisting of 200V hydrogen peroxide, in an approximate proportion of 3% gr/l., and this operation is effected at a temperature of between 40ºC and 60ºC for 15 to 30 minutes, after which the garments are washed again twice, 13 and 14, after which the final or finishing phase 15 begins, where the garments are immersed in a water bath 16, in which a softening agent 17 has been dissolved, consisting of an animal matter, preferably fatty acid or any amphoteric substance, in an approximate proportion of 2% of the weight of the matter, and denatured alcohol, and this last bath is effected at a temperature of between 60ºC and 80ºC, for 10 to 20 minutes.
